

Patented July 24, 1928.

1,678,379

## UNITED STATES PATENT OFFICE.

GEORGE ALBERT CHAPMAN, OF FOREST HILLS, AND ELTOFT WRAY WILKINSON, OF QUEENS VILLAGE, NEW YORK, ASSIGNORS TO MINERALS SEPARATION NORTH AMERICAN CORPORATION, OF NEW YORK, N. Y., A CORPORATION OF MARYLAND.

### COAL BRIQUETTE AND PROCESS OF MAKING IT.

No Drawing.

Application filed March 17, 1926. Serial No. 95,456.

This invention relates to coal briquettes and processes of making them, and is herein illustrated in part as applied to the production of briquettes from high ash coal and 5 from coal ashes such as are found on city dumps.

In the briquetting methods hitherto used it has usually been deemed necessary to dry the coal in rotary driers until it contained 10 less than 1% of moisture. It has also been deemed necessary to limit the crushing of the coal to a minimum amount because it has been deemed necessary to keep the total surface of the coal particles as small as possible, thus reducing the amount of binder required to coat the surface of the particles. Coarse crushing has resulted in retaining in 15 the coarse particles much of the ash which would be mechanically freed by fine crushing and could then be separated by suitable methods of coal concentration. Such processes therefore cannot commercially convert the high-ash waste of coal mines into valuable fuels in competition with the good coal 20 generally marketed. Usually the hot, dry, coarse-crushed coal as it comes from the drier has been mixed with hot oil or tar or asphaltic binder in a mixer which had to be kept hot. The mixed hot material has 25 usually been cooled slightly, pressed in a briquette press and then baked in an oven to set the binder and drive off some of the volatiles from the binder.

The briquettes thus produced from American coals have usually proved unsatisfactory for the American market. Those containing upwards of ten per cent of oil or asphalt usually have been quite smoky, while those containing smaller amounts of binder 30 have been objectionable because the binder has failed to mix uniformly with the coal, some coal particles having too much binder and others having too little or none at all, resulting in a dusty briquette,—that is one 35 which goes largely into dust when it breaks, because the uncoated particles or insufficiently coated particles have no tendency to stick together. As a result the briquette loses its integrity in burning and the particles which 40 are practically unbound fall apart as dust. In domestic fires this dust falls through the grates, passing into the ash as unburned carbon, with the result that the ashes left 45 by burning the briquettes hitherto made

have frequently contained as much as 60% 55 of unburned carbon. Household ashes resulting from the burning of properly sized anthracite average only from 30 to 40% of unburned carbon.

Some methods of producing briquettes 60 have used inorganic binders which not only increased the ash content but also resulted in dusty briquettes which as above noted are wasteful and unsatisfactory.

According to the present invention these 65 and others objections are overcome. Moreover it is found possible to crush the coal fine and yet use a relatively small amount of binder. The process therefore is well adapted to produce valuable fuel from high 70 ash waste coal which can be crushed and concentrated as well as fine waste coal, both of which are now generally regarded as useless, and which generally have not been capable of profitable utilization in commercial 75 briquetting processes with American coals for the American market. The coal is usually crushed to finer than ten-mesh and frequently even to less than thirty-five mesh, depending on the quality and ash content of 80 the coal. This fine crushing frees many particles of coal from included or adhering ash, and thus facilitates the separation of the pure coal from the ash by the froth-flotation process. Where the coal is concentrated 85 by froth-flotation there is usually employed in this process a soluble mineral-frothing agent, such as cresylic acid, and also an oil, which for example, may be a tar oil or coke oven tar or topped petroleum. 90

The crushed coal with the flotation agents is agitated in sufficient water to make a freely flowing pulp with the result that the coal floats. If little oil has been used the separate coal particles are carried in bubbles which float in the form of a froth. If larger amounts of oil have been used the coal will become agglomerated and the agglomerates may be floated or may be sunk. 95

Usually it has been found preferable to 100 concentrate the coal by froth-flotation, thus enabling the purified coal to be separated from the bulk of the pulp by removing the floating coal, thus easily and economically separating the coal from the bulk of the 105 water of the pulp and from the ash which remains behind in the pulp water. It may be advantageous to concentrate the coal by

froth-flotation with a little oil and then add more oil to agglomerate the coal. This may reduce the water associated with the coal from say 200% to say 35%.

- 5 A large proportion of the oil necessary for binding purposes in the production of briquettes is often thus disseminated by agitation in the presence of water, thus effecting a uniform distribution of it on the surface of 10 the coal particles. Usually this extra oil has the advantage of facilitating the draining of the water away from the coal to be briquetted. The oil in some cases may be added in the form of emulsion, especially 15 with heavy oils, or tars which play the part of oils, and the emulsion may be made with laundry soap or other emulsifying agent before adding it to the pulp.

It has been found advantageous to add to 20 the aqueous pulp, in general, not more than about 2% or 5% of oil measured on the weight of the coal. The rest of the oily or other binding agent is usually mixed later with the dried or partly dried pulp, as in a 25 paddle or dough mixer. It is preferable that air or gas be present in the pulp when adding the binder to the pulp or causing the binder to coat the coal particles in the pulp.

One great advantage of adding a substantial part of the binder in the pulp so 30 that the coal is coated with it by agitation in water, is that all of the particles of coal seem to be almost uniformly coated with the binder and thus, in the presence of sufficient binder, are certain to adhere or stick 35 to each other and produce a practically dustless briquette. Moreover if the coal particles are well agglomerated by an oily material such as oil, tar or pitch, the coal particles 40 and the agglomerates become water-repellent and water runs away from the coated coal and from the agglomerates, and is practically free of coal.

Owing to the fact that the agglomerates 45 are water-repellent they may be drained by leaving them in heaps, although it is usually preferable to drain them by special draining appliances such for example as a cocoa matting in the form of a continuous belt. 50 Frequently the best results are obtained when the agglomerates are drained by means of a continuous suction or centrifugal filter. Sometimes it is possible to obtain the agglomerates of coal in the form of hard 55 shotlike granules, especially when the agitation is accompanied by a minimum of aeration. Such shotlike granules may be freed from water by centrifuging. The drying operation usually reduces the moisture contained to somewhere between 15% and 25%. 60 It is not found necessary to dry the agglomerates to the extent that has hitherto been deemed necessary in drying the materials for briquetting, but it is usually advantageous 65 to thereafter reduce the contained moisture,

either by heat or by pressure, to between 5% and 10%. The moisture may be expelled by pressing these agglomerates in a mold which is provided with narrow drainage openings or slots, since the agglomerates usually do not flow through such openings under pressures running up to two tons or more per square inch. The continuous screw press as of the type used for pressing oil from seeds may be used where large capacity is not required.

To produce a strong briquette from the agglomerates containing from one to five or sometimes more per cent of oily material, the oil-coated coal particle or agglomerates are 80 preferably mixed with a further quantity of binder, which may be melted or crushed pitch, or Mexican fuel oil, or any one of a large number of oily materials, or sulphite cellulose liquor residues. It will be noted 85 that these materials are substantially ashless. When coal particles are already oil-coated, either by this process or in other ways, there is little difficulty in uniformly coating them with a further quantity of oily 90 material. It has been found possible to mix in uniformly as little as two or three per cent additional oil in a paddle mixer or a dough mixer, either hot or cold depending upon the material, and in this way add the 95 amount of additional oil or oily material necessary to make good and uniform briquettes. For reasons of economy the total oil or oily material needed as binder to make good briquettes is kept as small as possible. For other reasons it has been found 100 advisable to keep the oily material below 10% to 12%, depending on the nature and coarseness of the coal. If more than that amount is used the coal has an oily feel, 105 and the unbaked briquette is too soft or mushy.

By properly adjusting the percentage of total binder and the percentage of moisture it has been found possible to obtain oil-coated coal particles which may be pressed into briquettes such as the ordinary pillow-briquettes that will not stick in the mold and will burn without breaking, will be dustless, and will bear handling by the automatic machinery used for the handling of coal.

Usually the briquettes after being formed in the molds are too soft to bear such handling, so they are usually hardened by baking at a temperature high enough to drive off some of the volatiles from the oil or other binder and yet not high enough to actually have the effect of producing coke. This renders the briquettes smokeless and odorless, 120 thus fitting them for sale in the most exacting markets. These results have been usually obtained by baking at temperatures above 300° F. and ultimately reaching about 500° F., but, generally, not much exceeding 125 130

the latter figure, although with some oils temperatures ultimately reaching 650° F. for a short time have been found to be most satisfactory. The baking of pillow-briquettes 5 reaching a thickness of an inch and a quarter has usually required one and one-half to two hours at the temperatures named. Single briquettes would sustain a crushing weight of 125 pounds when properly made.

10 It is found that briquettes of fine coal made as above described bear rough handling and burn better than do similar briquettes made of coarser coal. It has been found that a properly made domestic fire 15 of such fine coal pillow-briquettes will burn for twenty-four hours without apparent diminution of volume if left undisturbed, the porous ash framework or skeleton of the briquettes even at the bottom of the fire 20 keeping the fuel structure intact to the end. A fire like this is said to "last well". The cooled ashes, retaining the structural form of the original briquette, may be removed intact from the fireplace if handled cautiously. 25 These porous ash skeletons are easily crushed in the fingers, and, so far as observed, never form hard clinkers. The porous structure of the ash is such that air passes through it and burns out the carbon 30 of the coal so that the ash of briquettes burned in ordinary domestic stoves contained as little or two to three per cent of unburned carbon.

It was found that the different oily materials lost different amounts when the briquettes were baked and that relatively larger amounts of oily materials had to be used as binder where their volatile content was high. One sample of Mexican fuel oil lost 45% on baking.

40 It was found that some coals, and particularly the coal contained in the ashes of a city ash dump, did not take up enough oil or oily binder to form satisfactory agglomerates when agitated with the oil or oily binder in an aqueous pulp. It was found however that very good agglomerates could be made from such coals by adding a small amount, say one to three per cent of oil or 45 oily binder in the aqueous pulp. The further binder needed to make the briquettes was added by mixing in the additional binder with the fairly well dried agglomerates after removal from the pulp.

55 In recovering coal from the ashes of a New York city dump it was found that 25% to 30% of the ashes were fines which passed through 28 mesh screen and that these fines contained only a few per cent of coal. 60 Accordingly in most runs the fines were separated and rejected before grinding the ashes to 20 to 35 mesh preparatory to concentration.

Example 1.—Ashes from a New York 65 city ash dump screened and ground as above

were subjected to froth-flotation treatment with a suitable soluble frothing agent and with oily material, and then further oily material was added until about four or five per cent of oily material on the coal present 70 had been added. The partly drained wet concentrate contained about 32% of water. To 125 pounds of this concentrate (estimated to contain 100 pounds of solids) were added three pounds of finely ground pitch, 75 and the whole mixture was put through an Anderson expeller to reduce the water content to approximately ten per cent. The discharge from the Anderson expeller was further mixed and then briquetted. The resulting briquettes were baked at a suitable 80 temperature to make them practically smokeless. The finished briquettes, after cooling, were tested as to their water absorbing quality by immersion in water for about twenty 85 hours, and it was found that they absorbed only from 4½% to 6% of water.

Similar concentrates were agitated in a pulp in a standard minerals separation machine with between 4½% and 6½% of gas 90 house coal tar to form agglomerates. These were separated from much of the pulp water, by flotation, drained on burlap to further reduce the water to 32.8%, and then put through an Anderson expeller to reduce the 95 water to 9%. The resulting cake was fed directly to a Belgian roll briquetting machine and the resulting briquettes baked for one and one-half hours at about 500° F. The resulting briquettes were excellent. 100 After cooling they were tested by immersion in water for twenty hours and it was found they had absorbed from 1.7% to 1.9% water and showed no signs of disintegrating and were hard.

No determinations of ash content were made during this run, but such determinations were made in connection with another substantially similar run in which the ashes were passed over a sixteen-mesh screen to 105 separate out the fines. The material retained on the sixteen mesh screen was fed to a standard ball mill to be ground for flotation feed. The fine material was passed through a Dorr classifier adjusted so that the 110 overflow carried about two per cent of material larger than 35 mesh. This overflow constituted the mill tailings. The coarse material from the classifier passed to the ball mill along with the coarse material from the 115 sixteen-mesh screen and constituted the flotation feed. The flotation feed was ground in the ball mill so that 82% of it passed a 35 mesh screen and this contained 67.5% of ash.

The flotation was effected in a series of six minerals separation positive-feed sub-aeration vessels. The feed to flotation averaged about a ton and a half of solids per hour. To the material in the ball mill was 120 125 130

added an emulsion of Mexican fuel oil and water containing 45% of oil and a fraction of a per cent of laundry soap so that the oil fed amounted to 22.8 pounds per hour, together with about 1.1 pounds of cresylic acid per hour. A further 0.4 pound of cresylic acid per hour was fed to the first agitating vessel. The froth overflow from this vessel was fed to the fifth vessel in the series which, together with the sixth vessel, retreated the froth overflow. The tailings from the first vessel passed successively through the second, third and fourth vessels and the float therefrom was returned to the first vessel. The tailings from the sixth vessel were returned to and divided between the second and third vessels. Together with them was fed the overflow from the thickener in which the concentrate obtained from the fifth and sixth vessels was thickened. The flotation tailings from the fourth vessel were returned to the mill feed so that they passed through the sixteen-mesh screen and thereafter were treated as part of the raw material fed to the mill. The finished concentrate coming from the thickener contained 15% ash, which was reduced by filtration to 13%.

*Example 2.*—A high ash coal from St. Clair Coal Company, St. Clair, Pennsylvania, was ground in a ball mill so that all but 1.2% passed twenty mesh and 52.2% passed one hundred mesh. This was fed at the rate of from three-fourths of a ton to a ton and a half per hour to a minerals separation positive-feed subaeration machine of six cells. In the froth-flotation concentrating operation coal tar was added to the aqueous pulp at the rate of 7.6 pounds per hour together with pine oil at the rate of one quarter pound per hour, oxidized petroleum at the rate of 4.5 pounds per hour, cresylic acid at the rate of 3.6 pounds per hour, and a Mexican fuel oil emulsion containing about one third water and a very little soap, 1.47 pounds per hour. The original ash content of the coal, 27.5%, was reduced in the concentrate to 14.75%. This concentrate was agitated in a minerals separation standard machine and coke oven coal tar was added at the rate of 61.8 pounds per hour to form agglomerates. The agglomerates were overflowed and after filtration contained from 13.5% to 17.5% of water and were further dewatered by passing them through an Anderson expeller and the product was then mixed in a C. P. Day Company dough mixer with rather more than five per cent (computed on the coal present) of coke oven tar to make a total estimated binder of about nine per cent on the coal present in the agglomerates. The resulting material was made into briquettes which were baked at a suitable temperature. Tested in a standard type of domestic grate they were found

to be smokeless, they burned well, and they retained their shape during burning. The resulting ashes contained an average of two to two and one-half per cent of unburned carbon as contrasted with unburned carbon contained in the ashes of briquettes produced by prior art processes of about 50%.

*Example 3.*—High ash coal sludge from the Philadelphia and Reading Coal and Iron Company containing 27.75% of ash was fed to a standard type ball mill together with an emulsion containing Mexican fuel oil and a little laundry soap so that the oil fed amounted to 13 pounds per ton. With this material which was about 35 mesh or finer was fed 2.8 pounds of cresylic acid per ton so that there was a total feed of agents with the coal amounting to about 15.8 pounds per ton of material fed. Froth flotation was effected in a minerals separation positive-feed subaeration machine having eight cells. There was added at the first cell an additional 1.05 pounds of cresylic acid per ton of solids in the feed. The concentrate from the first two cells was fed to the seventh cell which, together with the eighth cell, was used as a cleaner. The tailings from the second cell passed through the third, fourth, fifth and sixth, being finally discharged as flotation tails, while the overflow from these latter cells was returned as middlings to the feed at the first cell. An additional 0.25 pound of cresylic acid per ton of solids in the feed was added at the fifth cell. The overflow from the eighth cell, constituted a cleaned concentrate. The concentrates were heaped up, the product of several similar runs being mixed together.

The ash content averaged about 11.6%. These were dried to about 7% of water and mixed in a dough mixer with additional 9% of Mexican fuel oil and then made into pillow briquettes in a set of 4-pocket Mashick briquetting rolls (Belgian type). The briquettes did not stick to the rolls and there was very little breakage of them. The briquettes were baked for one hour and a half at a temperature rising to something over 500° F. This yielded excellent briquettes which burned with so little smoke that it was not noticeable except upon careful examination.

Having thus described the invention, what is claimed is:

1. A baked briquette consisting of uncooked anthracite coal substantially passing 10 mesh and bound by a binder which consists largely of the residue of oil which is less than ten per cent on the coal, said briquette being adapted when burned in a deep mass in a grate to leave an ash containing less than ten per cent of unconsumed carbon and burning nearly or absolutely smokelessly and without substantial softening.

2. A strong coal baked briquette consisting

of uncoked fine anthracite coal bound together by a substantially ashless binder which is less than ten per cent on the coal, said briquette being substantially free of dust 5 when broken and burnable in a grate without substantial softening so as to leave an ash containing less than ten per cent of unconsumed coal.

3. A strong coal briquette consisting of uncoked fine anthracite coal containing less ash 10 than the impure coal from which it is made and bound together by a binder which is less than ten per cent on the coal, said briquette being substantially free of dust when broken 15 and burnable in a grate without substantial softening so as to leave an ash containing less than ten per cent of unconsumed carbon.

4. A strong coal baked briquette consisting of uncoked anthracite coal passing 10 mesh 20 bound together by a binder which consists largely of the residue of banked oil which is less than ten per cent on the coal, said briquette being burnable in a grate without substantial softening so as to leave an ash 25 containing less than ten per cent of unconsumed carbon, and absorbing less than seven per cent of its weight of water upon prolonged immersion in water.

5. The process of making coal briquettes 30 which consists in treating fine coal to coat it with a substantially uniform coating consisting of oily material in too small amount to serve as a binder, and then mixing the oil-coated coal, with further substantially ashless binder, and forming it into briquettes.

6. The process of making coal briquettes which consists in agitating an aqueous pulp of fine coal with an oily reagent to produce oil-coated coal agglomerates, separating the 40 agglomerates from the pulp and from excess water, mixing with further oily substantially ashless binder, and forming it into briquettes.

7. The process of making coal briquettes 45 which consists in agitating an aqueous pulp of the impure coal with a mineral-frothing agent and with an oily reagent to produce oil-coated coal particles, separating the particles from the pulp and from excess water, mixing with further substantially ashless binding material, and forming it into briquettes.

8. The process of making coal briquettes 50 which consists in agitating an aqueous pulp of impure coal with a mineral-frothing agent and with an oily reagent to produce floating oil-coated coal agglomerates, separating the agglomerates from the pulp and from excess water, mixing with further substantially ashless binder, and forming it into briquettes.

9. The process of making coal briquettes 55 which consists in agitating an aqueous pulp of fine coal with an oily reagent to produce oil-coated coal particles, separating the particles from the pulp and from excess water,

mixing with further substantially ashless binding material, forming the briquettes, and baking the briquettes at a temperature reaching the neighborhood of 500° F.

10. The process of making coal briquettes 70 which consists in agitating an aqueous pulp of the impure coal with a mineral-frothing agent and with an oily reagent to produce floating oil-coated coal particles, separating the particles from the pulp and from excess water and its contained ash, mixing with further substantially ashless binding material, and forming it into briquettes.

11. The process of making coal briquettes 75 which consists in agitating an aqueous pulp of the impure coal with a mineral-frothing agent and with an oily reagent to produce floating oil-coated coal particles, separating the particles from the pulp and from excess water and its contained ash, mixing with further substantially ashless binding material, forming the briquettes, and baking the briquettes at a temperature reaching the neighborhood of 500° F.

12. The process of making coal briquettes 80 which consists in agitating a pulp of the coal with an oily reagent adapted to serve as binder to produce floating agglomerates, overflowing the agglomerates from the pulp to separate them from most of the excess 85 water, further dewatering the agglomerates, mixing the agglomerates with further binder, and then forming the mixture into briquettes.

13. The process of making briquettes from 90 impure coal which consists in agitating a pulp of the impure coal with a mineral-frothing agent to produce a floating coal concentrate, agitating the coal concentrate with an oily reagent adapted to serve as 95 binder to produce floating agglomerates, overflowing the agglomerates from the pulp to separate them from most of the excess water, further dewatering the agglomerates, mixing the agglomerates with further binder, 100 forming the mixture into briquettes, and baking the briquettes.

14. The process of making coal briquettes which consists in agitating an aqueous pulp of impure coal with a mineral-frothing 115 agent to produce a floating concentrate supported by bubbles, adding oily material which is adapted to serve as a binder, and further agitating to produce agglomerates of oil-coated coal, removing from the agglomerates the excess water, mixing further binder with the relatively dry agglomerates, molding the briquettes, and baking the briquettes.

15. The process of making coal briquettes 120 which consists in agitating an aqueous pulp of impure coal with a mineral-frothing agent to produce a floating concentrate supported by bubbles, adding oily material 125 which is adapted to serve as a binder, and

further agitating to produce agglomerates of oil-coated coal, removing from the agglomerates the excess water, mixing further oily binder with the relatively dry agglomerates, molding the briquettes, and baking the briquettes.

16. The process of making coal briquettes which consists in agitating an aqueous pulp of impure coal with a mineral-frothing agent and with an oil to produce a floating concentrate supported by bubbles, adding more oily material which is adapted to serve as a binder, and further agitating to produce agglomerates of oil-coated coal, removing from the agglomerates the excess water, mixing further binder with the relatively dry agglomerates, molding the briquettes, and baking the briquettes.

17. The process of making coal briquettes which consists in agitating an aqueous pulp of impure coal with a mineral-frothing agent and with an oil to produce a floating concentrate supported by bubbles, adding more oily material which is adapted to serve as a binder, and further agitating to produce agglomerates of oil-coated coal, removing from the agglomerates the excess water, mixing further oily binder with the relatively dry agglomerates, molding the briquettes, and baking the briquettes.

18. The process of making coal briquettes from ashes which consists in separating out the finer ashes, grinding the coarser ashes to free coal particles from adherent ash, agitating an aqueous pulp of the ground ashes with a mineral-frothing agent and with an oily agent to produce floating oil-coated particles, separating the float from the pulp and from excess water and its contained ash, mixing with further substantially ashless binding material, forming the mixture into briquettes and baking them to produce almost or absolutely smokeless briquettes.

19. The process of making coal briquettes from ashes which consists in separating out the finer ashes, grinding the coarser ashes to free coal particles from adherent ash, agitating an aqueous pulp of the ground ashes with a mineral-frothing agent and with an oily agent to produce floating oil-coated particles, separating the float from the pulp and from excess water and its contained ash, mixing with further substantially ashless oily binding material, forming the mixture into briquettes and baking them to produce almost or absolutely smokeless briquettes.

In testimony whereof, we have affixed our signatures to this specification.

GEORGE ALBERT CHAPMAN.  
ELTOFT WRAY WILKINSON.